

Sept. 2, 1969

S. M. SHELTON ET AL

3,464,813

## REDUCTION AND PURIFICATION OF REACTIVE METALS

Filed Oct. 20, 1965

2 Sheets-Sheet 1



Fig. 2.



Fig. 1.  $\frac{26}{2}$   $\rightarrow$  2



Fig. 7.

Stephen M. Shelton  
Henry Gordon Poole  
INVENTORS  
BY

BY  
Kolisch & Hartwell

Attys.

Sept. 2, 1969

S. M. SHELTON ET AL

3,464,813

REDUCTION AND PURIFICATION OF REACTIVE METALS

Filed Oct. 20, 1965

2 Sheets-Sheet 2



Fig. 3.



Fig. 5.



Fig. 4.



Fig. 6.

Stephen M. Shelton  
Henry Gordon Poole  
INVENTOR:

BY  
Kolisch + Hartwell

Attys

3,464,813  
REDUCTION AND PURIFICATION OF  
REACTIVE METALS

Stephen M. Shelton and Henry Gordon Poole, Albany, Oreg., assignors to Oregon Metallurgical Corporation, Albany, Oreg., a corporation of Oregon

Filed Oct. 20, 1965, Ser. No. 498,500  
Int. Cl. C22b 53/00, 5/04

U.S. Cl. 75—84.4

9 Claims

## ABSTRACT OF THE DISCLOSURE

A method of producing a reactive metal by reducing in a retort a halide of the reactive metal with a reducing metal to form the reactive metal distributed as a bed within the retort with such bed containing reducing metal and reducing metal halide as impurities. Such impurities are removed by heating the metal to a temperature which is below the boiling point of the impurities, and sweeping the retort with an inert gas whereby the impurities in vaporous form are carried from the retort. The impurities are then condensed to form particles and removed from the inert gas.

This invention relates to the production of reactive metals such as titanium, zirconium, hafnium, etc., and more particularly to a method and means for reducing a reactive metal halide and purifying the resulting product.

In the production of metals such as titanium, it is common to reduce a halide of the metal with reducing metal such as magnesium, sodium, potassium, etc. Thus, titanium tetrachloride, a liquid, may be added over a period of time to a batch of molten magnesium contained in a closed retort, with a reduction reaction taking place according to the following equation:



In the reaction, a porous sponge is formed of titanium, and mixed with this sponge and beneath the sponge the by-product magnesium chloride. Ordinarily, the reaction which takes place is not stoichiometric, and only a portion of the magnesium present in the retort is reacted, such as 75–85% of the magnesium. By reacting less than all of the magnesium it is possible to inhibit the formation of titanium subchlorides such as  $\text{TiCl}_2$  and  $\text{TiCl}_3$ . After the reduction reaction, therefore, there will be found in the reaction vessel in addition to titanium and magnesium chloride minor amounts of titanium subchlorides and magnesium. Much of the magnesium chloride may be tapped off while in a molten state, but the titanium sponge that remains in the retort still contains a certain amount of entrapped magnesium chloride as well as pure magnesium. The sponge, therefore, must be subjected to a purification process to obtain a titanium metal product of high purity.

Further discussing general problems attending the manufacture of a reactive metal such as titanium, magnesium when it is reacted with titanium tetrachloride is in molten form and tends to float on the by-product salt magnesium chloride produced by the reduction reaction. Liquid titanium tetrachloride is added to the magnesium by allowing the tetrachloride to fall from a pipe onto a pool of molten magnesium. To obtain a fast rate of reaction, and maximum production under controlled conditions, it is desirable to have as large an area as possible of molten magnesium exposed to the titanium tetrachloride dropping down thereon. It is also important that the titanium sponge which forms within the reactor be maintained in as shallow a bed as possible, in order that

the separation of impurities from the sponge in a subsequent purification step be facilitated. The purification of titanium sponge is further promoted if the sponge is formed as a relatively porous nondense mass, as this results in a larger surface area being produced throughout the sponge, and greater exposure of the impurities sought to be removed from within the sponge.

Titanium sponge which forms within a retort clings to the sides of the retort introducing a problem of the removal of the sponge after the process is completed. It is advantageous, therefore, in apparatus used to produce titanium, that a construction be selected for the reaction retort that permits easy loosening of the sponge from the retort walls.

As a way of purifying titanium sponge, it has been proposed that impurities be distilled off by heating the sponge in a closed retort for a period of time while maintaining a vacuum in the retort. A number of problems are introduced by such a procedure, however, since distillation is done at elevated temperatures, with weakening of the walls of the retort, and the usual retort must be heated within a special vacuum furnace if the retort is to be prevented from collapsing. Furthermore, there is always the danger of a leak developing in the equipment, with the loss of the batch of titanium sponge being processed.

One general object of this invention is to provide an improved process for preparing and purifying reactive metals, which is highly reliable, and at the same time relatively economical to carry out.

A related object is to provide improved apparatus for preparing and purifying a reactive metal.

A more specific object is to provide an improved method for producing a reactive metal, which features the use of the same retort for the reduction of the metal and for its purification, and the same furnace for heating the retort to produce the operating temperatures required within the retort. A further feature of the method is the maintenance of a pressure condition within the retort which is atmospheric or nearly atmospheric pressure, whereby the furnace employed for heating need not be a vacuum furnace, and assurance is had that the retort will not collapse during the manufacturing process.

A further object is the provision of a method for producing reactive metals characterized by the use of an inert gas stream passed through a retort at substantially atmospheric pressure, for removing vaporized impurities, and a novel method of removing impurities from this inert gas stream upon such leaving the retort.

Another object is to provide an improved method of the type above indicated wherein an inert gas is circulated through a retort with heating of the retort to remove vaporized impurities, the circulated gas is cooled in a region outside of the retort, and a portion of the cooled gas is mixed with hot gas flowing from the return for the purpose of initially cooling the hot gas. Using the method outline, solidification of impurities takes place in a novel manner which facilitates the removal of these impurities from the inert gas stream.

A still further object is to provide novel apparatus and method for reacting a reactive metal halide and a reducing metal such as magnesium wherein a large area of the reducing metal in molten form is provided during the reaction, and a relatively shallow bed of reactive metal is produced during the process facilitating subsequent purification of the metal by vaporization of impurities. Using the process and apparatus contemplated, a relatively porous sponge product may be produced, having a relatively large exposed surface area distributed through the sponge exposing impurities contained in the sponge.

These and other objects and advantages are attained by the invention, which is described hereinbelow in conjunction with specific illustrations of the invention and the accompanying drawings, wherein:

FIG. 1 is a side elevation, somewhat simplified, showing a retort such as may be used in the process of the invention, with the retort mounted within a furnace;

FIG. 2 is an end elevation, taken along the line 2—2 in FIG. 1;

FIG. 3 is a top plan view, somewhat simplified, showing apparatus for cleansing gas which is circulated in the process of the invention;

FIG. 4 is a side elevation, with portions broken away along the line 4—4 in FIG. 3, illustrating in simplified form a cooler unit in the cleansing apparatus;

FIG. 5 is a side elevation, with portions broken away along the line 5—5 in FIG. 3, illustrating in simplified form a filter unit in the cleansing apparatus;

FIG. 6 is a cross-sectional view, taken along the line 6—6 in FIG. 5; and

FIG. 7 (first sheet of drawings) is a cross-sectional view, somewhat enlarged, taken along the line 7—7 in FIG. 1.

In carrying out a preferred embodiment of the invention, an iron retort is employed for reducing and then purifying the reactive metal halide taking the form of an elongated hollow cylinder, closed at opposite ends, and disposed with the axis thereof horizontal. In the drawings this retort is indicated at 10, and comprises a cylindrical shell 12 and end walls 14, 16 closing off the ends of the shell. Slightly above the base of the shell and within the retort is a horizontal, perforated iron plate or reactor grid 18. Titanium sponge forms over this reaction grid upon the reaction of metal halide and reducing metal.

Retort 10 is supported on cradle structure 20 mounted on car hearth 22. The car hearth has wheels 24 disposed under it, riding on rails 26. Thus the retort is movable into and out of a furnace indicated generally at 28.

Piping of various types is shown communicating with the interior of retort 10. Specifically, pipe 30 projecting from rear end wall 14 of the retort adjacent its base, and connecting with the inside of the retort at a point located beneath grid 18, is provided for tapping the retort and removing salt by-product produced in the reduction reaction. Connecting with the retort at points 32a, 32b and 34a, 34b are pipes 32, 34, both of which connect with a common pipe 33, utilized in circulating gas through the inside of the retort. Pipe 35 is a blow off pipe, and at 37 is shown a pipe used in evacuating and back filling the retort. Extending from end wall 16 is an outlet pipe 36 through which gas flows on leaving the retort. A pipe 38 communicates with the retort adjacent the top of shell 12, and this comprises a feed pipe for feeding reactive metal halide to the retort.

Furnace 28 comprises sides 52 and a top 54 made of refractory furnace lining. The sides are apertured as at 56 to accommodate gas burners which supply the heat for the furnace. Furnace doors 58, 60 (see FIG. 2), slide laterally of the furnace, and suitably apertured to accommodate the pipes extending out the back end of the retort, are provided adjacent the back end of the furnace to close this end off. Similar furnace doors such as the one shown at 64 (see FIG. 1) close off the front end of the furnace.

According to this invention, purification of the reduced reactive metal produced in the retort by the reduction reaction is carried out with atmospheric or close to atmospheric pressure within the retort whereby a vacuum furnace is not required and the same furnace may be used to heat the retort during purification as was used in the reduction process. Purification is preformed by vaporizing impurities, and then sweeping them from the retort by circulating an inert gas such as argon therethrough. The invention also contemplates a novel method

of cleansing the argon or other inert gas used in the sweep process, with impurities being condensed and forming as solid particles which are collected. In the drawings, the apparatus producing circulation of gas through the retort while the same is in the furnace, and cleansing of the gas with removal of impurities, is shown in plan in FIG. 3, and is designated generally at 70.

More specifically, suitably supported on a platform 72 which is outside the furnace, are three cyclone filter units, given the reference numerals 74, 76 and 78, and a cyclone cooler unit, given the reference numeral 80. Platform 72 has wheels 82 underneath it supporting it on rails 26, enabling movement of the platform along the rails. Thus, the filter units and cooler unit may be moved bodily together with the retort on moving of the retort out of the furnace.

Referring to FIG. 1, outlet pipe 36 which gas flows through on leaving the retort is jacketed directly adjacent the retort, at 86, to permit the circulation of cold water around the pipe whereby a water cooled condenser section is formed. A water inlet and water outlet for the condenser section are shown at 86a, 86b. Progressing from condenser section 86, outlet pipe 36 connects with a valve 84 which connects with the top of cyclone cooler unit 80 by way of pipe 85.

Connecting with pipe 36 between where the condenser section is located and retort 10 is a pipe 88 for feeding cool gas into outlet pipe 36. As will be described in greater detail later, by feeding cool gas into the gas leaving the retort, and by the provision of the condenser section for further cooling of the gas leaving the retort, a temperature is produced in the gas mixture flowing through pipe 36 low enough to produce solidification of impurities in the gas stream with such being carried along as particles entrained in the gas stream.

Cyclone cooler unit 80 comprises a hollow cylindrical casing portion 80a forming the top of the unit, and a hollow conically shaped casing portion 80b forming the bottom of the unit. Flow into the unit through pipe 85 is against the inner surface of cylindrical casing portion 80a. Cooling water may be circulated about the outside of casing portion 80b, with such water flowing through a cooling line 80c extending in helical turns about casing portion 80b. Additional cooling in the unit may be brought about by including a jacket such as that shown at 80d about cylindrical casing portion 80a permitting cooling water to be circulated about the outside of the casing portion.

The cyclone cooler unit and cyclone filter unit 74 are interconnected by a pipe 90. A cooling water coil 92 intermediate the ends of pipe 90 provides additional cooling of gas flowing to the filter unit. Such cooling is desirable in order that gas entering the filter unit be at a low enough temperature so as not to burn up or otherwise damage filter cloths provided in the filter unit.

The various filter units are similar in construction. Thus, and referring to FIGS. 5 and 6, each includes a casing having a conical base such as the one shown at 74a for unit 74, and also a cylindrical top such as the one shown at 74b for filter unit 74. Within the hollow casing is a leaf-type filter made of folds of a filter cloth, such as the one shown at 74c, depending from a shield such as the one shown at 74d. Flow of gas out of the unit can take place only through the folds of the leaf-type filter and thence out through an outlet such as is provided by pipe 94. Material filtered out by the filter unit collects at the base of the unit in housing portion 74a earlier described.

Pipe 94 which provides an outlet for gas from the first filter unit extends from the first unit to the second filter unit 76. Gas flow out from this unit is through outlet pipe 96 which extends to the third filter unit 78. The outlet from the third filter unit is provided by a pipe 98.

Downstream from the third filter unit pipe 98 connects with the inlet side of an impeller pump 100 driven by

a motor 102. Gas exhausted from the pump passes through a pipe 104, which pipe branches into two pipes 105, 106. One of these, namely, pipe 105, joins with pipe 88 previously described in connection with the feeding of cool gas to outlet pipe 36 extending from the retort. Pipe 106 connects with pipe 33 provided for circulating gas through the retort. Flow meters for indicating the rate of flow through the pipes are indicated at 108 and 110, and valves controlling flow through the pipes are shown at 112 and 114.

The feeding of cool gas into pipe 36 for producing initial cooling of the gas coming from the retort and condensing of impurities contained in such gas is an important feature of this invention. The cool gas, as should be apparent from the above description of the apparatus, is obtained by diverting part of the inert gas circulated by the pump after such gas has been cleaned so that while much of the gas after cleaning passes through the retort to sweep it and remove impurities, a good proportion of the gas bypasses the retort to return to the gas flowing from the retort in pipe 36 at a point located in advance of the condenser section provided at 86. The gas is introduced to outlet pipe 36 in a special manner, moreover, whereby a film of moving gas, at a relatively low temperature, is produced which extends about the inside of pipe 36 to envelope hot gas flowing from the retort. Thus, and referring to FIG. 7, pipe 88 which connects with pipe 36 extends in a tangential direction from its point of joinder with pipe 36, and gas flowing into pipe 36 from pipe 88 tends to flow around the inner wall of pipe 36 to produce a spiraling flow of cool gas within pipe 36 as indicated by the arrow in FIG. 7.

The result of the construction above described, and the process by which a portion of the gas after cleaning and cooling is bypassed to cool gas flowing from the retort, is that impurities condense as particles entrained in the gas stream, and these particles are carried along pipe 36 without collecting on the wall of the pipe thereby to clog it. Put in another way, what the invention envisions is a system of cooling wherein condensed particles are formed, and these are formed in a traveling gas stream in a region away from the wall of the pipe confining the gas. The particles once solidified are carried by the gas stream into the cooler and filter units to be separated, and thence collect in the bases of these units.

In the case of the manufacture of reactive metals such as zirconium and hafnium, the halide is a solid, the retort is initially charged with the solid halide as well as with a mass of reducing metal such as magnesium. Thus, in this manufacture, pipe 38 is not necessary for the addition of the tetrachloride. Reduction of the tetrachloride takes place by sublimation of the halide, with halide vapors traveling in the retort to the region of the reducing metal which is present in the retort on heating as a molten pool.

The operation of the apparatus described and the method of the invention contemplated will now be explained with reference to the production of titanium from titanium tetrachloride and using magnesium as the reducing metal.

Eight hundred pounds of magnesium was first charged in a retort three feet in diameter and approximately six feet in length. The retort was mounted as pictured with its longitudinal axis horizontal. The retort was closed after charging with magnesium, by welding the end walls in place over shell 12. Cleansing and circulating apparatus 70 was suitably joined with the retort, and the retort was then evacuated and filled with argon to produce a pressure of 1 p.s.i.g. within the retort. Evacuating and filling with argon was performed using pipe 37. This pressure was maintained throughout the reduction and purification steps.

The retort was then mounted within furnace 28, and the furnace doors then closed. The gas burners of the furnace were ignited, and the retort was heated with the temperature of the walls of the retort rising to about 800° C. (1472° F.). Titanium tetrachloride was then fed to the retort through pipe 38, at a rate of about 600-800 pounds per hour, until 3000 pounds of the tetrachloride had been added over a period of about 4½ hours. During the reduction reaction, the temperature of the walls of the retort was maintained within the range of about 850-900° C. (1562-1742° F.). Argon was bled from the retort through pipe 35 so as to maintain the pressure within the retort constant. After about 60% of the titanium tetrachloride had been added (and the lapse of about 2½ hours time), by-product magnesium chloride formed in the reduction reaction was drained from the retort through pipe 30. The reduction reaction was about 75% efficient, and resulted in the production of about 600 pounds of titanium sponge. Estimated to be contained in the sponge was about 80 pounds of unreacted magnesium and 85 pounds of magnesium chloride and subchlorides.

Upon the completion of the reduction reaction, and the draining of all free magnesium chloride and magnesium from the retort, motor 102 was energized to start pump 100. Cleansing and circulating apparatus 70, which previously had been evacuated and back filled with argon, was placed in operation by adjusting of the valves controlling the flow of gas through pipe 33 and by-pass pipe 88, to produce a sweep of argon gas through the retort with such then being recirculated through the filter units. Gas flowed through the retort at the rate of approximately 50 cubic feet per minute, and the same rate of gas flow was maintained through the by-pass pipe. A pressure on the downstream side of the pump of about 5 p.s.i.g. was sufficient to produce proper circulation of gas through the equipment.

During the circulation of gas through the equipment, the furnace was operated and a temperature of from about 950-1050° C. (1742-1922° F.) maintained in the walls of the retort. Water was circulated through the various cooling coils and condenser sections described. Gas flowing from the retort had an average temperature of about 1000° C. A temperature of about 600° C. was noted 40 in the gas traveling into the cyclone cooler unit, and gas traveling into the first cyclone filter unit had a temperature of about 150° C. With some additional cooling of the gas occurring as the same traveled through the other filter units, and some heating of the gas occurring on 45 such passing through the compressor (25-30° C.), a temperature of from 60-70° C. was noted in the gas which 50 flowed through by-pass pipe into condenser section 86.

Purification by vaporization and sweeping of the retort was continued for approximately 48 hours. During this 55 time magnesium, magnesium chloride, and subchloride impurities collected in the bottoms of the various units as particles. At the conclusion of the purification process, the furnace was shut off and the retort removed and cooled to room temperature. The retort was then opened, 60 to reveal a web of titanium sponge disposed over the reactor grid in a region extending up to about three or four inches below the middle of the retort. The sponge was relatively easily removed by forcing the web of sponge upwardly toward the middle of the retort (not that the 65 sides of the retort diverge from each other progressing upwardly toward the middle of the retort promoting loosening of the web). A relatively porous pure titanium sponge product resulted, containing not more than 0.1% chlorine.

In the process of manufacturing titanium just set forth, argon was employed as the inert gas. Titanium has also been prepared employing a process similar to the one just set forth save that the inert gas helium was substituted for argon. The use of helium as the inert gas has some 70 particular advantages. For one thing, having a lower

density than argon, less power is required in pumping the gas whereby it circulates through the system. Furthermore, helium being less dense than argon there is more mobility of the molecules within the system which results in such advantages as the minimizing of hot spots in the retort during the reduction reaction.

The method of the invention features a number of advantages contributing to the relatively efficient production of large quantities of titanium sponge, of requisite purity, which method is reliable, and economical to perform.

Thus, of particular importance is the fact that the retort used in the reduction reaction and in the purification step is the same retort, and this retort is heated to operating temperatures while residing in the same furnace. Removal of impurities during the purification step is produced by vaporizing of these impurities, and relies upon sweeping of the retort with an inert gas at approximately atmospheric pressure (which may be defined herein as within the range of from atmospheric pressure to about 10 p.s.i. above atmospheric pressure) for bringing of the impurities out of the retort. Because of the pressure condition in the retort, heating during the reduction and purification steps need not be done in a vacuum furnace, but a conventional furnace may be used. It should be remembered that with operating temperatures close to 2000° F., the metal in the walls of the retort becomes quite weakened, and in a system which relies upon a pressure inside the retort substantially different from atmospheric, a furnace is required to hold the retort which will enable the production about the outside of the retort of a pressure condition similar to the one inside.

Furthermore, by utilizing a vaporization process wherein the impurities are swept from the retort with gas at close to atmospheric pressure, chances of inadvertent leakage both inside the furnace, and in the purification equipment outside the furnace, are sharply minimized. In a process where large pressure differentials exist, chances of inadvertent leaks occurring are ever present, and should a leak develop, the result is the loss of the entire charge of metal being produced.

With the elongated cylindrical retort employed positioned with the longitudinal axis thereof horizontal, a relatively large area of molten magnesium extends over the top of the molten pool of the metal. This promotes the reaction of the magnesium with the titanium tetrachloride introduced to the retort. Further explaining, and referring to FIG. 2, it will be noted that the cross-sectional area within the retort of a plane such as plane A paralleling the longitudinal axis of the retort is substantially greater than the cross-sectional area within the retort of a plane at right angles to the retort's longitudinal axis. Coupled with the advantage of obtaining a large exposed area for reaction, is the feature that a relatively shallow bed of sponge is formed for a given amount of reactants. The shallow bed promotes better vaporization of impurities from the sponge during the purification step. Another advantage of the type of retort disclosed is that the reactor grid covers a relatively large area, and presents a large filtration surface through which the magnesium chloride formed in the reaction may pass. At the completion of the reaction, since the sponge product is below a horizontal plane passing through the middle of the retort, it is easily removed by being forced upwardly into a region of wider dimension than the region the product originally occupied.

The magnesium chloride is not drained from the retort until at least about 60% of the titanium tetrachloride has been added. This tends to produce a more porous sponge product. If the magnesium chloride is drained earlier, the level of liquid magnesium in the reactor (which floats on magnesium chloride) tends to remain low, and new sponge tends to be produced on the addition of titanium tetrachloride in the interstices of already formed sponge to produce a dense product. With a more porous

product, vaporization of impurities during the purification step is facilitated.

Although vaporization of impurities is promoted by heating the products in the retort, the walls of the retort must be maintained below a temperature of about 2000° F. This follows from the fact that iron and titanium form a eutectic at a temperature only slightly under 2000° F. (approximately 1085° C.), and if the reactor walls exceed this temperature, undesirable reaction of the retort walls with titanium results. It should be noted that with a reactor of the type contemplated positioned with the longitudinal axis thereof horizontal, there is a maximum of wall surface bounding the region where a high temperature reaction occurs during the reduction part of the process available to dissipate heat. This is an additional feature of the invention.

The invention further contemplates, in combination with the sweep system of withdrawing vaporized impurities from the retort, a unique method of removing impurities as particles from the gas utilized to sweep the retort. Thus, cyclone units have been described where the impurities separate as particles and collect at the bases of the units. Note also that a novel bypass of cool gas into the gas emanating from the retort is contemplated, producing initial cooling of the gas mixture and condensation of the impurities in such a manner that clogging of the outlet pipe for the retort is inhibited.

Earlier the use of helium was described as preferred where it is desired to minimize the power used by the pump in circulating the gas and where it is desired to have the most even temperature conditions within the system. It should be pointed out here that the sweep evaporation contemplated herein, whether it be performed by argon, helium or other inert gas, promotes better efficiency in the system wherever heating or cooling is a factor than is possible with a system which relies on vacuum conditions. Because of the presence of the gas, the transfer of heat is not entirely the result of radiation as is the case where a vacuum is present, but also takes place by reason of convection.

While an embodiment of the invention has been described together with a working example, it is appreciated that changes and variations are possible without departing from the invention. It is desired to cover all modifications and variations of the invention as would be apparent to one skilled in the art, and that come within the scope of the appended claims.

We claim:

1. In the process of producing titanium by the reduction of titanium tetrachloride with magnesium in a retort, the steps comprising:

providing a retort having a charge of magnesium therein in a furnace, adding titanium tetrachloride to the retort while maintaining the walls of the retort at an elevated temperature by operation of said furnace, whereby the titanium tetrachloride reacts with the magnesium to product titanium, withdrawing by-product magnesium chloride from the retort,

vaporizing impurities in the titanium by heating the walls of said retort to an elevated temperature with the same furnace used during the reaction of magnesium with titanium tetrachloride,

circulating inert gas through the retort while so vaporizing such impurities with such gas at a pressure which is approximately atmospheric, such gas on leaving the retort carrying impurities with it, cooling the inert gas in a region outside the retort to cause condensation of impurities, separating the condensed impurities from the gas and then returning the gas to the retort as the gas circulated through the retort.

2. The process of claim 1, wherein cooling of the inert gas is done in such a manner as to produce particles of

impurities carried in a gas stream, and such particles are separated from the gas stream by gravity means.

3. The process of claim 1, where cooling of the inert gas is performed by mixing gas leaving the retort with cooler inert gas from another source, with such mixing producing condensation of impurities while such are being carried along by the gas stream leaving the retort.

4. The process of claim 1, wherein impurities are condensed and solidified while being carried along in a gas stream leaving the retort, and the impurities are separated from the gas stream by filtration.

5. In the production of titanium by the reduction of titanium halide with magnesium in a retort and subsequent purification of the reduction product through vaporization of impurities therein, the improvement comprising:

introducing the magnesium and titanium halide into an iron walled retort and with heating of the retort reducing the titanium halide to produce a titanium product distributed as a bed within the retort which comprises free titanium and impurities comprising magnesium and magnesium halide, and after the production of such titanium product and with such distributed as a bed in the same iron walled retort removing the magnesium and magnesium halide impurities from the titanium product through the steps of:

heating the titanium product in the iron retort at a temperature above the melting point and below the boiling point of the impurities to cause vaporization of the impurities, with the walls of the retort not exceeding the eutectic temperature of iron and titanium,

circulating an inert gas through the retort with such gas approximately at atmospheric pressure,

removing impurities from the retort by mixing the vaporized impurities with such inert gas, whereby the impurities travel with the gas out of the retort as part of an inert gas stream, in a region outside the retort cooling the inert gas stream including such impurities to a temperature below the melting point of the impurities to condense the impurities and form solid particles thereof, and

separating the impurities when in particle form from the inert gas stream.

6. The process of claim 5, wherein at least partial cooling of the inert gas stream is performed by mixing with the gas stream on such leaving the retort cooler inert gas substantially free of impurities.

7. The method of claim 6, wherein particles carried in the gas stream are removed by filtration.

8. The method of claim 6, wherein the cool inert gas comprises circulated gas which bypasses the retort.

9. In the process of producing titanium by the reduction of titanium tetrachloride with magnesium in a retort, the steps comprising introducing into the retort magnesium and titanium tetrachloride and heating the retort to an elevated temperature whereby the titanium tetrachloride reacts with the magnesium to produce titanium, withdrawing by-product magnesium chloride from the retort,

vaporizing impurities in the titanium by heating the retort to an elevated temperature which is above the melting point of the impurities but below the boiling point of the impurities,

circulating inert gas through the retort while so vaporizing such impurities with such gas at a pressure which is approximately atmospheric, such gas on leaving the retort carrying impurities with it, cooling the inert gas leaving the retort in a region outside the retort to cause condensation of impurities,

separating the condensed impurities from the gas, and then returning the gas to the retort as the gas circulated through the retort.

#### References Cited

##### UNITED STATES PATENTS

|           |           |                 |                 |                 |
|-----------|-----------|-----------------|-----------------|-----------------|
| 2,982,645 | 5/1961    | Olson           | -----           | 75—84.5         |
| 3,158,671 | 11/1964   | Socci           | -----           | 75—84.5 X       |
| 2,205,854 | 6/1940    | Kroll           | -----           | 75—84.5         |
| 2,663,634 | 12/1953   | Stoddard et al. | -----           | 75—84.5         |
| 2,745,735 | 5/1956    | Byrns           | -----           | 75—84.5         |
| 2,766,113 | 10/1956   | Chisholm et al. | -----           | 75—84.5         |
| 40        | 2,772,875 | 12/1956         | Levy            | ----- 75—84.5 X |
|           | 2,778,726 | 1/1957          | Winter et al.   | ----- 75—84.5   |
|           | 2,817,585 | 12/1957         | Winter.         |                 |
|           | 2,992,098 | 7/1961          | Boozenny et al. | ----- 75—84.5   |
| 45        | 3,252,823 | 5/1966          | Jacobson et al. | ----- 75—84.5 X |

L. DEWAYNE RUTLEDGE, Primary Examiner

H. W. TARRING, Assistant Examiner

U.S. Cl. X.R.

50  
75—84.5